

# UNITED STATES PATENT OFFICE.

AARON MENDLESON, OF ALBANY, NEW YORK.

## COATED CAUSTIC-ALKALI BALL.

SPECIFICATION forming part of Letters Patent No. 229,161, dated June 22, 1880.

Application filed September 10, 1879.

*To all whom it may concern:*

Be it known that I, AARON MENDLESON, of the city of Albany, State of New York, have invented a new and useful Improvement in the 5 Manufacture of Caustic-Alkali Balls, of which the following is a specification.

The nature of my invention consists in providing an extra thickness of coating material at the sprue-point of the ball, the extra thickness being a seal in the form of a boss.

In the manufacture of alkali balls the fused alkali is cast in metallic molds similar to bullet-molds, and the end of a short wire is often inserted into the ball at the sprue-hole while 15 the alkali is still melted in the mold. The wire thus being cast into or attached to the ball serves as a convenient handle or carrier of the ball in the subsequent operation of dipping in the coating material. When a carrier- 20 wire is not used there is also an irregularity of form of the ball at the sprue-point, which may be either an irregular nib or a depression. After the dipping in the coating, whether in the use of the carrier-wire or other device, the 25 irregularity at the sprue-point is often a cause of a failure in protecting the alkali from the injurious action of the air.

It is the practice, as soon as the ball is 30 coated, to nip off the wire close to the coating and to pour upon the sprue-spot some of the melted coating material, with the intent to protect the weak spot; but this device is not effectual, for the reason that the melted material being poured upon a prominence, and there 35 being no guide or restraint to the flow, it results that the larger part of melted material goes down and away from the sprue spot and adheres where it is not desired, the defect is not remedied, and the symmetrical form of the 40 ball is destroyed.

I find that a thin covering of the sprue-spot is not sufficient, and especially in the case where the wire device is employed the air penetrates a thin coating to the wire, oxidizes 45 and expands it. It results from this expansion

of the wire that cracks in the coating originate at the sprue-spot, and in a short time these cracks may creep under and through the whole coating. The air with its moisture and carbonic acid reaches the alkali through these 50 cracks, and the alkali dissolves and runs away. Such a ball is said to "leak." A leaky ball will destroy sound balls or other valuable goods with which it may be brought in contact.

To secure complete protection at the sprue-spot I provide thereupon a thick and symmetrical coating. Having placed the ball upon a suitable rest or stand, the ball having its sprue-spot upward, I lay upon it a heavy metal ring, so as to inclose the sprue-spot and to 60 serve as a curb and mold for the melted coating material. I pour the melted coating material upon the sprue-spot until the space inclosed by the ring is filled. When the material is cold the curb molding-ring is lifted off, and the operation is finished. The ring may be an 65 inch or less in diameter and about one-fourth of an inch high. The inner surface of the ring should not be cylindrical, but conical or sp' 70 ical, the diameter at top being less than at the bottom.

The boss of my invention, in addition to being a complete preventive of the leaking originating at the sprue-spot, is a pleasing addition to the form of the ball, and may be made 75 highly ornamental.

The accompanying drawing shows, in section, a coated alkaline ball, A, with the projecting boss C and the mold-ring B B.

What I claim is—

A coated alkali ball or block having a symmetrical sealing-boss which extends beyond the general contour of the ball, said boss forming a part of the coating, and being placed over and upon the sprue-spot, as described.

AARON MENDLESON.

Witnesses:

JAMES H. HUNTER,  
WILLIAM H. LEWIS.